

# UNITED STATES PATENT OFFICE.

ROBERT ABBOTT HADFIELD, OF LONDON, ALEXANDER GEORGE MACKENZIE JACK, OF SHEFFIELD, AND ISAAC BERNARD MILNE, OF TOTLEY, ENGLAND.

## MANUFACTURE OF ARMOR-PIERCING PROJECTILES.

1,310,075.

Specification of Letters Patent. Patented July 15, 1919.

No Drawing,

Application filed June 28, 1915. Serial No. 36,886.

To all whom it may concern:

Be it known that we, ROBERT ABBOTT HADFIELD, ALEXANDER GEORGE MACKENZIE JACK, and ISAAC BERNARD MILNE, subjects of the King of Great Britain and Ireland, residing at 22 Carlton House Terrace, London, Rock-hills, Brincliffe, Sheffield, county of York, Cross Grove House, Totley, county of Derby, England, respectively, have invented

10 new and useful Improvements in the Manufacture of Armor-Piercing Projectiles, of which the following is a specification.

This invention has for object to produce armor piercing projectiles, particularly of 15 large diameter, say of twelve inches and upward, that shall be better adapted than those heretofore commonly used to completely perforate thick hard faced armor plates without becoming broken up, or broken to 20 such an extent as to interfere with their subsequent desired action.

For this purpose an armor piercing shell according to the present invention is made of suitable steel, such as nickel chromium 25 steel, and subsequently treated in such a manner that the head or ogival forward portion of the shell is of different degrees of hardness varying say from a ball hardness of from about 600 to 700 at the pointed 30 front end portion or zone through successive rearward zones of about 500, 400 and 300 ball hardness, the zone having a ball hardness of about 400 terminating rearwardly say round about the forward portion of the 35 cavity in the shell and the zone having a ball hardness of about 300 extending farther rearward for a short distance around the shell cavity, the remaining rearward portion of the shell having a ball hardness 40 under 300.

In the production of such a shell, made say of nickel chromium steel, the shell after being formed to shape, as by casting it solid and then, after suitably annealing it, by 45 pressing it to shape in a suitable press, is hardened and tempered by subjecting it to two separate treatments of which the first consists in heating the shell all over in a suitable furnace to a hardening temperature, 50 the point of the projectile being protected from direct contact with the heating medium in a known manner to prevent overheating thereof and then dipping the shell point downward to its base end in a cooling medium, for example oil, where it is left

until cold. The second or tempering treatment consists in heating the base portion of the shell to a suitable tempering temperature while its pointed end portion is immersed point downward, to a suitable 60 depth in water, after which it is partially cooled and then immersed or quenched outright in a cooling medium, for example water.

The temperatures to which the shells are 65 heated, the depths and durations of immersion and other details can be variously modified to suit different sizes of shells and the character of the steel of which they are made.

According to one example, carried out with a twelve inch shell having a length of about thirty-four inches and made of nickel chromium steel having the following approximate composition, namely carbon .6 to .7%; nickel 2 to 3% and chromium 2 to 3%, for example carbon about .66%, nickel about 2.52% and chromium about 2.31%, the shell was heated all over to a hardening temperature while its point was protected from direct contact with the heat so that the external shoulder portion of the shell had a temperature of about 915° C. to 920° C., the inner surface or core adjacent to the shoulder portion being found to have, in 80 the example given, a temperature of about 900° to 905° C., the point a temperature of about 890° C., and the base a temperature of about 780° C. The shell thus heated was then hardened all over by dipping it in oil 85 to its base end and holding it there until practically cold, the cooling being effected from the exterior alone, that is to say without admitting any cooling medium to the interior of the shell. The hardened shell 90

was afterward subjected to a second or tempering treatment consisting in heating the base portion thereof in a furnace to a temperature of about 670° to 705° C.; its interior or core having a temperature of 100 about 605° C. while its pointed end portion was immersed to a depth of about eight and a half inches in water kept cold. The shell was then allowed to cool down in the furnace to a base temperature of about 320° C. to 105 300° C. and an internal or core temperature of about 290° to 255° C. whereupon it was quenched outright in water. When thus treated, the pointed portion of the shell for about the first ten inches of its length had 110

a ball hardness of 600 and over, the weight of this portion comprising about 12% of the total weight of the projectile, the ball hardness varying from 600 at ten inches 5 from the point to 418 at fourteen inches, 311 at 18 inches and 241 at the base end of the shell.

According to another example carried out with a fourteen inch shell having a length 10 of about fifty-two inches and made of nickel chromium steel having the following approximate composition, viz., carbon 69% nickel 2.53% and chromium 2.70%, the shell was heated all over while its point was protected from direct contact with the heat so that the external shoulder portion of the shell had a temperature of about 930° C., the inner surface or core adjacent to the shoulder being found to have in this example 15 a temperature of about 900° to 905° C., the point a temperature of about 875° C. and the base a temperature of about 850° C. The shell thus heated was then dipped in oil to its base end and held in that position 20 until cold, the cooling being effected wholly from the exterior inward. The hardened shell was afterward subjected to a second or tempering treatment consisting in heating the base to a temperature of about 700° 25 C., its interior or core having a temperature of about 630° C. while its point was immersed for about a depth of eight inches in water kept cold. The shell was then allowed to cool down in the furnace to a base 30 temperature of about 310° C. and a core temperature of about 255° C. and then quenched outright in water. In this case the first eight inches had a ball hardness 35 of 652 and over, this portion constituting 40 about 6% of the weight of the shell, the hardness decreasing to the base where it was about 262.

From the foregoing examples it will be seen that the temperatures to which the 45 various parts of the shell can be heated and the manipulation of the shell can be variously modified without departing from the essential features of the invention.

The second or tempering treatment can 50 advantageously be applied to shells subjected to a first or hardening treatment other than that hereinbefore described. Also, the feature of protecting the hardened point of a projectile during the second 55 or tempering treatment by immersion in water or other medium kept cold, as by frequent renewal or otherwise, is a feature of considerable importance and applicable generally in the tempering treatment of projectiles.

The above mentioned temperatures are given by way of example only. As hereinbefore indicated however, the temperatures may be varied upward or downward to suit 60 circumstances.

What we claim is:—

1. The process of heating an armor piercing shell which consists in heating the shell all over to a hardening temperature, then hardening the projectile all over by immersion, point downward, in a cooling medium of the same character throughout and allowing it to remain therein until substantially cold and subsequently subjecting the shell 70 so hardened to a tempering treatment. 75

2. The process of treating an armor piercing projectile which consists in heating the shell all over to a hardening temperature while protecting the point from direct contact with the heating medium, and then 80 dipping the shell point downward in a cooling medium and leaving it there until practically cold.

3. The process of treating an armor piercing projectile which consists in heating the 85 shell all over to a hardening temperature while protecting the point and then dipping the shell to its base in a cooling medium and leaving it there till practically cold.

4. The process of producing an armor 90 piercing projectile having the head of different degrees of hardness varying at the pointed front end from about 700 to 600 ball hardness, diminishing in hardness to about 400 at about the front end of the cavity, 95 about 300 around the cavity and the rearward portion under 300, which consists in heating the projectile all over to a hardening temperature the external shoulder portion about 900° C. or over, the point about 900° 100 C. or a little under, and the base about or under 800° C., and then dipping the shell in a cooling medium and leaving it there till practically cold.

5. The process of heating an armor piercing shell which consists in heating the shell all over to a hardening temperature, then dipping the shell point downward to base in a cooling medium of the same character throughout and leaving it there until comparatively cold, the cooling being effected 105 from the exterior inward without special internal cooling.

6. The process of treating an armor piercing projectile which consists in heating the shell all over to a hardening temperature, then dipping the shell point downward in a cooling medium and allowing it to remain 115 there until practically cold and subsequently subjecting the hardened shell to a tempering treatment consisting in heating the base or body portion of the shell to a suitable tempering temperature while the point of the shell is kept cool, and afterward cooling the shell. 120

7. The process of treating an armor piercing shell which consists in heating the shell all over to a hardening temperature then dipping the shell to base in a cooling medium and allowing it to remain therein until it is 130

practically cold, then heating the base of the hardened shell to a suitable tempering temperature while the point of the projectile is immersed in a cooling medium, then allowing the shell to partially cool and thereafter quenching the shell outright in a cooling medium.

8. The herein described process of hardening an armor piercing projectile which consists of producing a projectile of the approximate composition:—carbon about .6 to .7, nickel about 2. to 3., and chromium about 2. to 3., heating the projectile all over to a hardening temperature while protecting the point, and then dipping the projectile to its base in a cooling medium and leaving there till cold.

9. The herein described process of hardening an armor piercing projectile which consists in heating the shell to a hardening temperature, then dipping the projectile in a cooling medium and allowing it to remain there till cold, and then tempering the projectile by heating the base to a tempering temperature while protecting the point and then cooling.

10. The process of treating an armor piercing projectile which consists in heating the shell all over to a hardening temperature while protecting the point from direct contact with the heating medium, and then dipping the shell point downward in a cooling medium and leaving it there until cold, then tempering the projectile by heating the base to a tempering temperature, while its pointed end portion is immersed in water, then partially cooling and then quenching outright in a cooling medium.

11. The process of treating an armor piercing projectile which consists in heating the shell all over to a hardening temperature while protecting the point and then dipping

the shell to its base in a cooling medium and leaving it there till cold, and then tempering the same by heating the base to a tempering 45 temperature while protecting the point, then partially cooling and then quenching in water.

12. The process of producing an armor piercing projectile having the head of different degrees of hardness varying at the pointed front end from about 700 to 600 ball hardness, diminishing in hardness to about 400 at about the front end of the cavity, about 300 around the cavity and the rear- 55 ward portion under 300, which consists in heating the projectile all over to a hardening temperature, the external shoulder portion about 900° C. or over, the point about 900° C. or a little under, and the base to about 60 or under 800° C., and then dipping the projectile in a cooling medium and leaving it there till cold, and then tempering the projectile by heating the base in a furnace to a temperature of about 670° to about 705° 65 C., its interior having a temperature of about 605° C., while its pointed end is immersed to about eight and one half inches in water kept cold, then permitting the projectile to cool in the furnace to a base temperature 70 of about 320° C. to about 300° C. and a core temperature of about 290° C. to about 255° C., and then quenching the same outright in water.

In testimony whereof we have signed our 75 names to this specification in the presence of two subscribing witnesses.

ROBERT ABBOTT HADFIELD.  
ALEXANDER GEORGE MACKENZIE JACK.  
ISAAC BERNARD MILNE.

Witnesses:

Wm. Cross,  
Wm. O. Brown.